

J. S. HEALY.  
PRINTER'S BLANKET.  
APPLICATION FILED NOV. 11, 1913.

1,147,942.

Patented July 27, 1915.



Attest:  
John S. Healy  
Washington Reiter

John S. Healy, Inventor:  
by Wm. J. Dolan Atty

# UNITED STATES PATENT OFFICE.

JOHN S. HEALY, OF NEW YORK, N. Y., ASSIGNOR TO GEORGE L. WILLSON, OF NEW YORK, N. Y.

## PRINTER'S BLANKET.

1,147,942.

Specification of Letters Patent.

Patented July 27, 1915.

Application filed November 11, 1913. Serial No. 800,245.

*To all whom it may concern:*

Be it known that I, JOHN S. HEALY, a citizen of the United States, and a resident of the borough of Brooklyn, city of New York, county of Kings, State of New York, have made certain new and useful Improvements in Printers' Blankets, of which the following is a specification.

The invention relates to printers' blankets 10 and methods of making the same, and has for an object to provide an improved construction of the character referred to which shall be highly efficient and economical in operation.

15 Other objects of the invention will be apparent from the following description.

The invention consists in the novel methods, improvements, features of construction, and combinations of elements hereinafter 20 more fully set forth.

In the accompanying drawings, which is referred to herein and forms a part hereof, is illustrated an embodiment of a feature of the invention, the same serving in connection with the description more fully to explain the invention.

The drawing is a perspective view of a portion of a printer's blanket constructed in accordance with the invention and the 30 proportions are distorted in order better to show the construction.

Referring now in detail to the drawing, there is illustrated a preferred embodiment 35 of the invention made in accordance with one feature thereof. This comprises a body of yielding material which may be made of various materials and in different ways. Preferably, a composition is made having elasticity and at the same time being impervious to oil. The preferred composition includes glue; glycerine, which prevents hardening of the glue and forms therewith an elastic compound and one that is not injuriously affected by the ingredients commonly used in printer's ink. To these are added gum arabic and china clay which add body to the composition and prevent undue softening by heat; and a small quantity of antiseptic, as formaldehyde, will be useful.

40 While these materials may be mixed in various proportions, the preferred composition includes four parts glue, five parts glycerin, one-half part gum arabic, and one-half part china clay. To this preferably is added a 45 sixty-fourth part of formaldehyde.

In the best embodiment of the invention a fabric 1, as flannel, having a nap on both sides, is impregnated with this composition, and to this impregnated fabric is attached on each side a suitable fabric 2 without a 60 nap, as muslin, the composition forming a layer 3 between each two strips of fabric.

According to another feature of the invention, on the member thus produced there is superposed in operation another member 65 4 of yielding material. This member may be made of various materials. It has been found, for example, that for certain kinds of work a sheet of the cloth known as "tympan" may be used, in which case the 70 composition member is made thicker than would ordinarily be the case. It will be noted that the composition member may be made of any desired thickness by varying the number of layers of impregnated fabric 75 or the amount of composition used. When a tympan sheet has been used, it may be lifted from the composition member and replaced with another sheet, if desired. On other kinds of work a strip of felt may be super- 80 posed upon the first or composition member, and, while the felt member will become attached to the first member because of its texture and of the heat and friction due to operation of the press, yet it may be detached from the first member, when desired. 85 Moleskin, for example, may also be used.

The preferred method of making the printer's blanket of the invention is as follows: A composition is made of the desired 90 ingredients, the desired fluidity being obtained by adding water, as say three parts to the specific mixture described. In a suitable vessel containing the composition is laid the fabric with the nap on one or both 95 sides and the fabric is thoroughly impregnated with the composition. It is then removed and placed between two sheets of fabric, as muslin, and the three sheets are pressed between rollers or in a press. Upon 100 said member there is preferably superposed in operation a sheet of yielding material, as fabric.

A printer's blanket, constructed in accordance with the invention will be very durable 105 and economical in operation and at the same time highly efficient, and will possess many other advantages which will be apparent to those skilled in the art.

The invention in its broader aspects is 110

not limited to the precise constructions or proportions of parts shown and described nor to any particular constructions by which the same has been or may be carried into effect nor to the precise steps or sequence of steps in the method of making the same which has been described, as many changes may be made in details without departing from the main principles of the invention or sacrificing its chief advantages.

I claim:

1. A printer's blanket comprising a body of yielding material impregnated with a compound including four parts glue, five parts glycerin, and one-half part china clay.
2. A printer's blanket comprising a body of yielding material impregnated with a compound including four parts glue, five parts glycerin, one-half part gum arabic, and one-half part china clay.
3. A printer's blanket comprising a body of yielding material impregnated with a compound including four parts glue, five parts glycerin, one-half part gum arabic, one-half part china clay, and one sixty-fourth part formaldehyde.
4. A printer's blanket including a layer of felt, a plurality of layers of woven fabric, and a layer of glutinous, fabric-impregnating compound indissoluble in oil and interposed between the woven fabrics and adhered to by the felt.
5. A printer's blanket including a layer of felt, a layer of muslin, a layer of woven fabric, and a layer of glutinous, fabric-impregnating compound indissoluble in oil and interposed between the muslin and woven fabric, and with which the felt, muslin and woven fabric adhere.
6. A printer's blanket including a glutinous, fabric-impregnating compound indissoluble in oil and including glycerized glue,

gum arabic, and china clay, a layer of felt on one side of and adhering to said compound, and a layer of adhering woven fabric on the opposite side thereof.

7. A printer's blanket including a nap-carrying element, a woven fabric, and an interposed oil-resisting compound including glycerized glue and china clay impregnating said nap-carrying element and adhering to the woven fabric.

8. A printer's blanket including a layer of nap-carrying fabric, a sheet of woven fabric, and an interposed oil-resisting, felt-impregnating compound comprising glue, glycerin, gum arabic and china clay.

9. A printer's blanket including a layer of felt, a sheet of woven fabric, and an interposed oil-resisting, felt-impregnating compound comprising glue, glycerin, gum arabic, china clay and formaldehyde.

10. A printer's blanket including a layer of felt impregnated with an oil-resisting compound comprising four parts of glue, five parts of glycerin, a one-half part gum arabic, and a one-half part china-clay, and a layer of woven fabric adhering to said compound.

11. A printer's blanket including a layer of felt, a layer of muslin, a layer of flannel, and layers of a glutinous, fabric-impregnating compound indissoluble in oil and interposed between the felt and muslin and between the muslin and flannel, respectively, and with which felt, muslin and flannel the compound adheres.

In testimony whereof, I have signed my name to this specification, in the presence of two subscribing witnesses.

JOHN S. HEALY.

Witnesses:

GEORGE PALMER,  
GEO. L. WILLSON.

Copies of this patent may be obtained for five cents each, by addressing the "Commissioner of Patents, Washington, D. C."